

April 12, 1938.

F. MARANDE

2,113,895

STEEL TAPPET CONSTRUCTION

Original Filed July 29, 1935



INVENTOR

Frank Marande.

BY

Harnett, Dickey, Pierce & Hann

ATTORNEYS

## UNITED STATES PATENT OFFICE

2,113,895

## STEEL TAPPET CONSTRUCTION

Frank Marande, Saginaw, Mich., assignor to  
Eaton Manufacturing Company, Cleveland,  
Ohio, a corporation of Ohio

Original application July 29, 1935, Serial No. 33,  
723. Divided and this application December  
12, 1936, Serial No. 115,502

8 Claims. (Cl. 123—90)

This invention relates to the construction of steel valve tappets for internal combustion engines, and is a division of my co-pending application, Serial No. 33,723, filed July 29, 1935, for 5 Steel tappet constructions, and assigned to the same assignee as is the present application. Tappets are used to transmit the thrust of the engine cam to the valve stem and require a hard, wear resisting face for contact with the cam but 10 at the same time the face must not be so brittle as to be easily fractured under impact.

Cast iron cam engaging heads or wear portions have previously been employed in tappet constructions, and while they provide a good 15 wearing surface, they have the disadvantage of being more fragile and brittle than steel. Increased engine speeds and increased valve loads have made it necessary and desirable to provide in a tappet construction a head member which 20 has wearing qualities practically comparable to cast iron, but which is stronger, lighter and less subject to fracture under impact.

Various steel constructions of tappets have also been proposed, but all of these require a 25 considerable amount of forging and a deformation and reworking of the hard steel of the facing or head member. Steel head members or facings having the desired wearing qualities are so hard that they are not easily machined or worked by 30 forging. According to the present invention, a construction is provided in which forging or machining of the face or head member is substantially eliminated so that the disadvantages of reworking a hard steel material and of causing 35 development of flaws and inequalities of distribution during such forging operation are eliminated.

The principal object of this invention is to 40 improve the art of tappet construction.

Another object is to provide a tappet construction in which the metal or alloy of both the 45 facing or head member and of the body member of the tappet are sensitive to the same heat treating and quenching process to obtain the desired hardness of both members and to eliminate stresses between such parts.

It is also an object of the invention to provide 50 an extremely light weight tappet construction which includes considerably less metal than conventionally employed, but at the same time provides the desired strength and resistance to wear and fracture under impact.

A further object is to provide a tappet construction having a relatively thin facing or head 55 member supported only adjacent the outer mar-

gins thereof so that it will flex sufficiently to afford a cushioning effect and allow the tappet to follow the surface of the operating cam therefor and substantially eliminate bounce of the tappet relative to the cam shaft. 5

Other objects, features and advantages will become apparent from the following description and the appended claims.

For the purpose of illustrating the genus of the invention, typical concrete embodiments thereof and preferred method of fabricating the same are shown in the accompanying drawing, in which:

Figure 1 is a side elevation, partly in section, 15 of the body portion of a tappet made in accordance with the principles of this invention;

Fig. 2 is a top or bottom plan of the head portion of a tappet shown in Fig. 1;

Fig. 3 is an end view, in elevation, of the head portion shown in Fig. 2; 20

Fig. 4 is a view similar to Fig. 1 of the body and head portions of the tappet assembled in a welding jig for the initial welding operation.

Fig. 5 is a view similar to Fig. 4 showing the tappet after the welding operation has been completed; 25

Figs. 6 and 7 are views similar to Figs. 4 and 5 and showing, respectively, the tappets prior to and after the forging operation for simultaneously effecting extrusion of the head portion and 30 upsetting of the body portion have been completed;

Fig. 8 is an elevation, partly in section and similar to Fig. 3, of a modified form of tappet body mounted in a welding fixture and with a head portion assembled thereon prior to the welding operation. 35

Figs. 9 and 10 are views similar to Figs. 4 and 5 of a further modified form of tappet body prior to and after the head portion has been welded thereto; and 40

Fig. 11 is a side elevation of a completed tappet of the type illustrated in Figs. 9 and 10.

Referring to the drawing, and more especially to Figs. 1 to 8, inclusive, the body portion of the tappet consists of a tubular member 1, preferably composed of steel or an alloy thereof, performed by machining or other desired mechanical operations to provide a thickened and flanged upper end portion, the upper surface of which is beveled to provide a line contact portion 3. The underside of the flange is also slightly beveled as indicated at 4. The lower end of the tubular member is provided with a reduced bore which is threaded as indicated at 5, in Fig. 1, to receive 55

an adjusting screw or stud which may be threaded in or out of the lower end of the tappet for adjustment purposes. The lower end of the tubular member 1 is reduced in outside diameter as indicated at 6, in Fig. 1, and provided with wrench flats formed on diametrically opposite sides thereof for receiving a wrench during adjusting operations of the tappet. The tubular member 1 is made of a free cutting steel, such as standard specification S. A. E. 1335 steel which has been found to be an especially suitable material. This steel contains approximately 0.30-0.40% carbon, 1.35-1.65% manganese, 0.15-0.30% silicon, 0.05% maximum phosphorus, 0.07-0.15% sulphur and the balance iron. This steel hardens readily to about 40-50, Rockwell scale C, when heated and at a temperature of about 1500-1520° F. and quenched in oil. This steel affords good resistance to wear and is readily machined and forged.

A wear piece or head member adapted to be attached to the body member 1 is shown in Figs. 2 and 3 and consists of a preformed annular disc of wear and impact resisting metal or alloy. Standard specification S. A. E. 52100 steel constitutes the preferred material of the disc or head member 8. This material is composed of approximately 0.95-1.10% carbon, 0.20-0.50% manganese, 1.20-1.50% chromium, 0.15-0.30% silicon, 0.03% maximum phosphorus, 0.035% maximum sulphur, and the balance iron. Other steels or steel alloys may be used in construction of head portion 8 such as 3% tungsten tool steel, a tool steel known by the trade name "Ketos", and standard specification S. A. E. 6150 steel. One form of 3% tungsten tool steel has approximately 1.20-1.40% carbon and 3.00-5.00% tungsten, the balance being principally iron, while a quite similar form of tungsten tool steel has approximately 1.35-1.50% carbon, from 0.50-1.00% chromium, from 0.20-0.30% vanadium, and from 3.50-5.00% tungsten, the balance being principally iron. "Ketos" steel has approximately 0.90-1.00% carbon, about 1.50% manganese, 0.50-0.60% chromium and 0.15-0.20% vanadium, the balance being principally iron. Standard specification S. A. E. 6150 steel contains approximately 0.45-0.55% carbon, 0.50-0.80% manganese, 0.80-1.10% chromium, 0.18% vanadium, 0.04% maximum phosphorus, 0.045% maximum sulphur, and the balance iron. While this steel does not produce quite as great hardness as the standard specification S. A. E. 52100, it is noted that the wearing qualities of the head member may be improved by cutting said head members from bar stock in which rolling operations during the production of the bar stock have caused the grains of the steel to be arranged axially of the piece. When such head members are employed in a tappet the wear occurs across the ends of the grains of the steel rather than in the direction of the fibers of the material. Standard specification S. A. E. 52100 steel has somewhat more chromium and about twice the carbon content of the S. A. E. 6150 steel, which probably accounts for its superior hardness and wear resisting qualities or characteristics when heat treated. It is preferred to employ the latter steel for the head member 8 since it affords the necessary hardness and wear resisting qualities. The 3% tungsten tool steel also affords the necessary hardness and in this characteristic is slightly superior to the "Ketos" steel. Standard specification S. A. E. 52100 steel is, however, more economical to produce than the tungsten tool steel or "Ketos"

steel, and is particularly desirable for the present tappet since its heat treating characteristics are essentially the same as that of the steel employed in the body portion of the tappet. It will be noted that in each instance, a steel alloy containing a metal of the chromium family, i. e., the chromium-molybdenum-tungsten-uranium family, is used and in certain instances, other hard metals such as manganese and vanadium are also employed to harden the steel alloy. It will also be noted that in each instance, a steel alloy contains about 0.55-1.50% carbon. When the carbon content is at or near the lower of such limits, it is necessary to employ, about 5 to 8% of the hard metal in the alloy. With a carbon content from about 0.90-1.50%, the hard metal content may be reduced to from about 1 to 5%, thus effecting an economy in the cost of the material used for the cam engaging portion.

The disc 8 may be formed by any desired method such as punching from sheet or bar stock, stamping, casting, or otherwise fabricating the same to substantially the desired ultimate size of the tappet head when the disc is made of one of the above described materials or a similar material which affords the desired wearing and impact resisting qualities. Where the wear resisting quality of the material selected for the tappet head is not otherwise quite sufficient, the disc may be forged from bar stock so that wear of the head member or wear piece will take place across or transverse to the end grain of the steel rather than in the direction of the fibers of the material in order to obtain the desired wear resistance. A disc 8 of substantially the desired ultimate size of the tappet head is indicated in full line in Figs. 2 and 3. This disc, however, may be made smaller than the ultimate head size but of greater thickness, as indicated by the dot and dash outline in Fig. 3, so that the discs may be spread and thinned out in the forging operation during formation of the tappet.

Referring to Figs. 4 to 7, inclusive, the method of joining the body and head members 1 and 8, preformed as above described, consists in mounting the body 1 in a hollow welding electrode 9 and then positioning the head or disc 8 on the flange 2 of the body member with the underside of the disc 8 in contact with the thin line contact portion 3 formed at the upper edge of the flange 2. The second welding electrode 10 is then brought against the upper surface of the head member or disc 8 and the welding circuit closed. The welding current passes through the thin line contact portion 3 and melts the metal of the adjacent side of the body and head member. The welding is continued until the welded joint between the head member and the body member extends substantially across the widest portion of the flange 2, as shown in Fig. 5. This is in the nature of a progressive welding operation and is carried out in the manner described so as efficiently to utilize the welding current and to secure as broad a homogeneous weld between the parts as is possible with the possible area of contact between such parts. The provision of the thin line contact between the head and body members causes the metal of the flange 2 to melt with considerable rapidity first at the point of contact which affords the path of least resistance, and causes pre-heating of adjacent parts of the flange 2 and the head member 8, so that when the two parts come into full contact, as shown in Fig. 5, a substantially uniform weld will

be completed across the greatest width of the flange 2.

Another method of welding head and body portions may involve the use of a modified form of tubular body 1' shown in Fig. 8, such body member being provided with a flange 2' so formed that the thin line contact portion 3 lies at the diametrically outer margin of the flange 2'. Although an acceptable weld may be obtained

10 with the form of flange shown in Fig. 8, the most desirable practice is to form the flange so that the line contact portion is at the diametrically inner margin of such flange. It is also possible to obtain an acceptable weld by so forming the flange 2 that the line of contact between it and the head member will initially occur at a point intermediate the diametrically inner and outer margins of the flange 2. This, however, may necessitate additional machining operations 15 which are not desirable because of cost.

After the head member 8 has been welded to the body member 1 or 1', as above described, the assembled article, if desired, may be reheated to a desirable forging temperature and placed in a die member 12, as shown in Fig. 6. This die member is provided with a longitudinal cavity of a size adapted correctly to receive that portion of the body 1 or 1' below the flange 2 or 2', and with an enlarged cavity of a size corresponding 20 to the ultimate desired size of the head member 8. The lower surface of this upper cavity is inclined toward the reduced cavity which receives the lower part of the body 1 or 1', the inclination being at a degree slightly less than the bevel 4 on the 25 under side of the flange 2 or 2'. The inclination of this die cavity may be regulated to control to some extent the direction of displacement or upsetting of the metal of the flange 2 or 2' in the forging operation. After the assembled construction has been placed in the die member 12, it is 30 engaged by a punch 13, and flange member 2 or 2' and the head member are forged together as shown in Fig. 7. The forging operation causes the flange 2 or 2' to be deformed in both directions with reference to the major axis of the tubular body, broadens the contact between the under side of the head member 8 and the body member 1 and reworks the initial weld between the head and body members. This not only strengthens 35 the weld but also broadens the bearing between the head member 8 and flange 2. The forging operation may also be carried to such an extent as to extend the support of the flange 2 or 2' outwardly towards the edges of the head member 40 50 and also radially inwardly of the walls of the body member 1 or 1' so that the thickened walls of the tappet body afford a greatly increased area of support at the point where the greatest strain occurs during use of the tappet. The extent to 55 which extrusion of the metal of the head member 8 into the tubular end of the body member 1 or 1' and extrusion of the metal of the flange 2 or 2' outwardly toward the outer margin of the head member 8 may be controlled by regulating the travel of the punch 13. The purpose of such extrusion of metal is to secure an embracing engagement between the head member and body at the welded joint.

After the forging operation has been completed, 60 only such finishing operations as tapping or otherwise threading the reduced bore 5, final heat treatment, rough and finish grinding the stem or body portion 1 of the tappet and finish grinding the end face of the head portion 8 remain to be done. The above indicated heat

treatment involving a 1500-1520° F. quench in oil gives the body portion 1 of the tappet a hardness of about 40-50, or above, Rockwell scale C, for the major portion of such body member, and gives the head portion a hardness of about 55, or more, on the same scale. The forging operation may be accomplished cold or with such heat as remains in the unit after the welding operation, although it is preferable to re-heat the assembly before forging.

Reference may now be had to Figs. 9, 10 and 11 in which is depicted a method of making a barrel type tappet. Body 21 of said tappet is preferably made by casting and is composed of a suitable steel or alloy which is capable of hardening by heat treatment. The body portion 21 is cast so as to provide a hollow tubular portion with a relatively large bore 22 through the major portion thereof and to provide relatively thin walls so as to eliminate as much weight as possible. 10 A reduced bore 23 is provided at one end of the tappet so that one end of such body portion will have relatively thicker walls which may be internally threaded to receive an adjusting screw 25 for adjusting the clearance between the end 20 of the valve stem of an internal combustion engine and the tappet. A lock nut 26 may be provided for maintaining such adjustment. Openings or windows 24 may be provided in the walls of the body portion 21 for further lightening the 30 weight of a tappet for distributing lubricant between the walls of the tappet and the guide therefor and admitting air for cooling purposes to the interior of the tappet. The body portion 21 is preferably cast in a permanent mold and may 35 be of a steel or alloy such as a material composed of approximately 2.75-3.5% carbon, 0.40-1.10% manganese, 1.70-2.60% silicon, 0.20-0.30% phosphorus, 0.115% sulphur, and the balance iron. This material is sensitive to the same heat treatment as the head portion 8', corresponding to the head portion 8 of the previously described embodiment, and composed of essentially the same material as the head portion 8, to produce substantially the same hardness of head portion and 40 body portion as previously indicated. The upper surface of the body portion 21 is beveled to provide a thin annular line contact portion 27 to facilitate progressive welding of the head and body portion of the tappet and to produce uniform 45 welds in the manner above described. The body member 21 is mounted in a hollow electrode 9' and the head member 8' is then positioned on the upper end of the tappet body with the under side of the head member in contact with the line 50 contact portion 27. A second welding electrode 10' is then brought against the upper surface of the head member 8' and the welding circuit closed. The progressive welding operation is carried out in the manner above described sufficiently to utilize the welding current and secure as broad 55 and homogeneous a weld between the parts 8' and 21 as is possible with the available area of contact between such parts.

The tappet may then be subjected to a heat 60 treatment for hardening the same by reheating the tappet so as to obtain the proper hardness and then quenching in oil when at a temperature of from 1500 to 1520° F. The tappet may then be finish ground and the adjusting screw 25 and 65 lock nut 26 assembled thereon. The thickness of the cam engaging disc 8' is preferably approximately equal to, or but slightly greater than the thickness of the peripheral walls of the body portion 21. The disc 8' is supported only adjacent 70 75

the periphery thereof by the body portion 21 so that the disc will flex sufficiently to afford a cushioning effect during operation of the tappet, and the tappet will follow closely the surface of an operating cam and eliminate bounce relative to the crank shaft.

As many changes may be made in the above described constructions, and many apparently widely different embodiments of this invention could be had without departing from the spirit thereof, it is intended that all matter contained in the above description or shown in the accompanying drawing shall be interpreted as illustrative and not in a limiting sense.

15 16. What is claimed is:

1. As an article of manufacture, a heat-treated tappet including a body portion integrally bonded to a cam engaging portion, said body portion being composed of a steel consisting of substantially 20 1.35-1.65% manganese, 0.30-0.40% carbon and the balance principally iron, and said cam engaging portion being composed of a steel consisting of 25 0.20-0.50% manganese, 0.95-1.10% carbon, 1.20-1.50% chromium and the balance principally iron, so that when both of said portions are heated and at a temperature of about 1500 to 30 1520° F. are quenched in oil, stresses between the joint portions are substantially eliminated and the body portion has a hardness of from 40 to 50, Rockwell scale C, and a cam engaging portion has a hardness of about 55, Rockwell scale C.

2. A tappet construction comprising a tubular body portion of medium carbon steel integrally bonded to a substantially disc shaped wear portion 35 of a steel alloy containing a metal of the chromium family, the grain of the steel of said wear portion being disposed substantially parallel with the axis of said tubular body portion.

3. A tappet comprising a hollow tubular steel 40 body and a steel cam engaging portion in the form of a disc having a thickness not materially greater than the thickness of the walls of said body portion, said disc being secured to and supported by said body portion only adjacent its 45 periphery so as to flex sufficiently during operation of the tappet to afford a cushioning effect whereby the tappet follows closely the surface of the operating cam therefor.

4. As an article of manufacture, a heat treated 50 tappet including a body portion integrally bonded to a cam engaging portion, said body portion being composed of a medium carbon steel and said cam engaging portion being composed of a steel alloy selected from a group of steels consisting of 55 standard specification S. A. E. No. 52100 steel, "Ketos" tool steel, and 3% tungsten tool steel, both of said portions being sensitive to a heat treatment involving heating said portions to a temperature above 1500° F. and at a temperature 60 of from about 1500 to 1520° F. quenching in oil to produce a hardness of about 55 Rockwell scale C for the cam engaging portion and a hardness of 40 to 50 Rockwell scale C for the major portion of said body portion.

5. As an article of manufacture, a heat treated tappet including a body portion integrally bonded to a cam engaging portion, said body portion being composed of a steel consisting of substantially

1.35-1.65% manganese, 0.30-0.40% carbon, and the balance principally iron, and said cam engaging portion being composed of a steel alloy selected from the group of steels consisting of standard specification S. A. E. No. 52100 steel, 5 "Ketos" tool steel and 3% tungsten tool steel, both of said portions being sensitive to a heat treatment involving heating said portions to a temperature above 1500° F. and at a temperature of from about 1500 to 1520° F. quenching in oil 10 to produce a hardness of about 55 Rockwell scale C for the cam engaging portion and a hardness of 40 to 50 Rockwell scale C for the major portion of said body portion.

6. As an article of manufacture, a heat treated 15 tappet including a body portion integrally bonded to a cam engaging portion, said body portion being composed of a medium carbon steel and said cam engaging portion being composed of a steel alloy including from 0.55-1.50% carbon, from 1 20 to 8% hard metal selected from a group of hard metals consisting of chromium, tungsten, molybdenum, uranium, manganese and vanadium, and the balance being principally iron, both of said portions being sensitive to a heat treatment involving 25 heating said portions to a temperature above 1500° F. and at such temperature quenching in oil to produce a hardness of about 55, Rockwell scale C, for the cam engaging portion and a hardness of 40 to 50, Rockwell scale C, for 30 the major part of said body portion.

7. As an article of manufacture, a heat treated tappet including a body portion integrally bonded to a cam engaging portion, said body portion being composed of a steel consisting of substantially 35 1.35-1.65% manganese, 0.30-0.40% carbon, and the balance principally iron, and said cam engaging portion being composed of a steel alloy including from 0.55-1.50% carbon, from 1 to 8% hard metal selected from a group of hard metals 40 consisting of chromium, tungsten, molybdenum, uranium, manganese and vanadium, and the balance being principally iron, both of said portions being sensitive to a heat treatment involving heating said portions to a temperature above 45 1500° F. and at such temperature quenching in oil to produce a hardness of about 55, Rockwell scale C, for the cam engaging portion and a hardness of 40 to 50, Rockwell scale C, for the major part of said body portion.

8. As an article of manufacture, a heat treated tappet including a body portion integrally bonded to a cam engaging portion, said body portion being composed of a medium carbon steel and said cam engaging portion being composed of a steel alloy including from 0.55-1.50% carbon, from 1 to 8% hard metal selected from a group of hard metals consisting of chromium, tungsten, molybdenum, uranium, manganese and vanadium, and the balance being principally iron, both of said portions being sensitive to a heat treatment involving 60 heating said portions to a temperature of about 1500° F. and at such temperature quenching in oil to produce a hardness of above 50, Rockwell scale C, for the cam engaging portion and a hardness of above 40, Rockwell scale C, for the major part of said body portion.

FRANK MARANDE.